

July 16, 1935.

R. B. McCauley

2,007,977

METAL WITH PHOSPHIDE CASE AND METHOD OF PRODUCING SAME

Filed Feb. 29, 1932

2 Sheets-Sheet 1



Inventor  
Roy B. McCauley

Witness:

R. B. Dawson

By Wilkinson, Harley, Byron & Knight  
Atts.

July 16, 1935.

R. B. McCauley

2,007,977

METAL WITH PHOSPHIDE CASE AND METHOD OF PRODUCING SAME

Filed Feb. 29, 1932

2 Sheets-Sheet 2



Witness:  
R.B. Dawson.

Beij Wilkinson Hayley Byron & Knight

Inventor,  
Roy B. McCauley,

Patented July 16, 1935

2,007,977

# UNITED STATES PATENT OFFICE

2,007,977

## METAL WITH PHOSPHIDE CASE AND METHOD OF PRODUCING SAME

Roy B. McCauley, Chicago Heights, Ill.

Application February 29, 1932, Serial No. 595,849

11 Claims. (Cl. 148—7)

The object of the present invention is to produce upon an article made of iron, steel and some other metals known to react with phosphorus to form phosphides and by reaction upon the metal itself, a case that will render the article substantially immune to attack from acids, alkalies and other chemical influences.

While the principle has long been realized that alloying phosphorus with iron and steel increases the resistance of the metal to surface corrosion and other chemical attack, it has not to my knowledge hitherto been applied in a manner to successfully develop, upon an article of such metals, a case consisting of an alloy of phosphorus with the metal, of such depth and such union with the body of non-phosphorized metal as will insure permanency of the case and complete exclusion of corroding influences from the metal.

The present invention resides in a simple, efficient and comparatively inexpensive method of procedure whereby an existing article of iron, steel or some other metal may, without injuring the article by excessive temperature, be converted into a new article of manufacture by having developed upon it a phosphorus alloy case of such inherent chemical formula and inherent character; of such penetration into the body or depth of case, and with such diffusion of merger with the portion of the article that is not alloyed with phosphorus, that the case will not be readily removed by abrasion, spalling or flaking off, and it will hermetically exclude from the body of the metal, corrosive and other reacting influences to which phosphidized metal is immune.

The invention is characterized by the conditions, among others, that the alloying of phosphorus with the metal of the article is carried out in a manner to cause the protective case to exist in the form of a phosphide of the metal of the article, as distinguished from a phosphate or other form of combine. This phosphide is developed at a temperature that is so far below the critical temperature of the metal of the article as to exclude any distortion of the design of the article or any injury to its metal structure. The phosphide-forming conditions are such that they may be maintained for any desirable period of time by way of regulating the depth to which the reaction penetrates and consequent thickness of the resultant case, thus enabling the conversion of the outer areas of the metal to any desired extent short of weakening the physical strength of the body. Penetration resulting from continued reaction of the phosphorus with the metal of the article does not proceed so uniformly

throughout the affected area as to leave any accurately defined plane of demarcation between the phosphide and the non-phosphorized metal, but leaves, rather, a condition that I shall herein term "diffused merger" of the thus alloyed and non-alloyed portions, so that spalling off, chipping, or flaking of the substantial thickness of phosphide does not occur. The procedure lends itself readily to introduction of the element of pressure as an influence upon the reaction to such extent as may be desired. And an aqueous protecting environment may conveniently be used when it is desired to employ metallic phosphorus as the source of alloying ingredient. The aqueous protection may be in the form of water if low pressure and temperature below boiling are sufficient in any particular case, or in the form of steam when an aqueous protection under high pressure and temperature is desirable. The use of this aqueous protection for pure phosphorus reagent may continue throughout the process or be continued only during the time necessary to charge the treatment chamber with the goods and reagent, with exclusion of air, or may be omitted altogether; and in any event, vaporization of the phosphorus itself in the hermetic treatment chamber, by the heat of the treatment, may be relied upon to develop internal pressure desired in influencing the reaction.

In many instances it will be desirable to use relatively high temperatures (less than the critical temperature of the metal of the article) and in so doing to employ as a source of reagent, phosphorus released by reduction, under the heat of the process from one of its compounds, or still more conveniently prepared in the form of phosphine. Generally speaking, the depth of the protective case will be influenced by the time during which the reaction is continued, and this circumstance renders desirable the use of a phosphorus source, such as phosphine, which can be fed into the treatment chamber as long as may be desirable. The temperature maintained during the reaction will strongly influence the rate of the reaction.

In carrying out the method of the invention, and producing the new article of the invention, several procedures may be followed.

One procedure would be to enclose an article, made of iron or steel or some other metal appropriate to the procedure, in a chamber and subject it to the action of molten phosphorus submerged in water heated up to 212° F.; and this may be varied to the extent of having the chamber closed tightly enough to confine steam

under substantial pressure and thereby subject the work to a temperature materially above 212° F.

According to a second procedure, the metal article may be enclosed with metallic phosphorus in a container capable of withstanding high pressure and such pressure developed by heating and vaporizing the phosphorus; the degree of pressure being dependent on the size of the chamber and the quantity of phosphorus introduced. And in this second procedure the phosphorus may be initially protected by water until the heating chamber can be hermetically sealed, the water being in an open container from which it will readily disappear by evaporation early in the procedure leaving the phosphorus subject to vaporization, or the phosphorus may be initially protected by introducing it in the form of a cartridge or sealed in a suitable destructible envelope which would be ruptured by the pressure of the phosphorus when vaporized within it, thus releasing the phosphorus for reaction as the temperature is developed.

According to a third procedure, the phosphorus source may be phosphide of a metal having a less affinity for phosphorus than has the metal of which the article is made, the metal phosphide being packed around the article to be cased and the transfer of the phosphorus being induced by the heat of the procedure.

A fourth procedure embodying the method of the invention and producing the new article of manufacture, and one which is preferred because of the great flexibility which it offers in temperature and pressure of the reacting environment, as well as facility for continuing the supply of the reagent, and thereby controlling the time during which the reaction is continued, consists in placing the article to be cased in a chamber, for instance, a tube, one end of which has a venting tube submerged in water to a depth that will impose a desired back pressure within the chamber, and the other end of which said chamber is in communication with a container or generator of phosphine (PH<sub>3</sub>); the said tubular chamber being located within a heater capable of developing a desired temperature in the chamber. In this fourth procedure, the reaction can be regulated by not only the temperature maintained, but largely, and particularly as to rapidity, by controlling the input of the phosphine. Through means of this fourth procedure involving the method of the invention, and with a reaction of phosphine through a period of about one half an hour, upon an article made of steel I have produced a case having a depth of one sixty-fourth (1/64th) of an inch and consisting of an iron phosphide corresponding to the formula Fe<sub>2</sub> P (which is 15.63% phosphorus), and have tested such article with its said case by immersing it in a 10% solution of hydrochloric acid for a period of thirty days and found that the article did not lose appreciably in weight, and its case was firmly secure against chipping off.

Also, by the above described fourth procedure or embodiment of the method of the invention, I have treated articles made of steel having a carbon content in one instance of three one-hundredths of one per cent (.03%), and in another instance one per cent (1.00%) and, by such treatment lasting over a period of about four hours and using phosphine as the reagent, formed upon said articles phosphide cases having a depth of about one thirty-second (1/32nd)

of an inch, corresponding to the formula Fe<sub>2</sub> P<sub>3</sub>, which is 45.45% phosphorus. In one of these latter experiments, a piece of one per cent (1.00%) carbon steel, in developing its phosphide case of Fe<sub>2</sub> P<sub>3</sub> formula (45.45% phosphorus), was subjected to treatment for about five hours.

In these last-named instances of treating low and high carbon steels, the specimens were pieces of rolled steel and the scale of iron oxide formed on the steel in rolling was not removed in advance but was reduced in the procedure. The iron reacted with the phosphorus of the PH<sub>3</sub> gas, leaving in the tubular chamber an atmosphere of hydrogen which, in turn, reacted with the iron oxide scale and left the latter upon the specimen in the form of iron according to the formulas 2PH<sub>3</sub> plus 4Fe yields 2Fe<sub>2</sub>P plus 3H<sub>2</sub>, and 3H<sub>2</sub> plus Fe<sub>2</sub>O<sub>3</sub> yields 2Fe plus 3H<sub>2</sub>O; the resulting iron being then converted to iron phosphide by the incoming PH<sub>3</sub> gas as 2PH<sub>3</sub> plus 4Fe yields 2Fe<sub>2</sub>P plus 3H<sub>2</sub>.

If at any time during the operation of the fourth procedure an excess of phosphine is delivered to the tubular chamber, it will be manifested by self ignition of the phosphine on reaching atmosphere of room temperature in escaping from the water into which the venting tube is dipped, and this converts it into phosphoric acid (P<sub>2</sub>O<sub>5</sub>) by the reaction of 2PH<sub>3</sub> plus 4O<sub>2</sub> yields P<sub>2</sub>O<sub>5</sub> plus 3H<sub>2</sub>O. If the bubbles coming through the water into which the venting tube is dipped do not take fire on reaching atmosphere, it may safely be assumed that the atmosphere in the reaction chamber is hydrogen and the phosphine entering the chamber is not excessive.

In the accompanying drawings, four suggestive designs of apparatus convenient for practicing the invention are shown by way of illustration—

Figure 1 showing, in side elevation, a small installation for casing small articles;

Figure 2 showing, partly in side elevation and partly in longitudinal section, an installation with the reaction chamber designed for treating long articles, such as pipes and tubes, enclosed in a furnace.

Figure 3 showing, partially in longitudinal section, an apparatus in which the reaction chamber is in the form of a wheeled car running on a track and employing an extraneous source of heat; and

Figure 4 showing in side elevation, partly in section, an apparatus in which an electric resistance element is used as the source of heat.

Referring to Figure 1, 1 represents a commercial cylinder of phosphine gas, 2 a commercial cylinder of inert gas such as hydrogen, 3 a three-way valve receiving gas from cylinders 1 or 2 and discharging the same through pipe 4 into reaction chamber 5 contained within a furnace 6, which may be equipped with usual accessories such as heat source 7, furnace door 8, pyrometer tube 9 and gauge 10. From the reaction chamber 5 extends a venting pipe 11 which dips into a body of water 12 a distance sufficient to develop a desired back pressure in pipe 11 and thereby regulate the pressure under which reaction in chamber 5 proceeds. This apparatus may also be provided with loading and unloading table 13.

After an apparatus such as illustrated in Figure 1 is assembled for phosphorizing, that is to say, the articles to be cased are enclosed in the reaction chamber 5, the air should be washed out of the apparatus by means of a current of hydrogen from the container 2, or it may be ordinary illuminating gas, in order to insure a

reducing instead of an oxidizing atmosphere in the chamber. This being done, gas from cylinder 2 is cut off and phosphine (PH<sub>3</sub>) from cylinder 1 is introduced into the reaction chamber 5, and while the temperature of the furnace 6 is kept up to a degree just above that needed for the reaction, say, a temperature of from 300 to 800° F., the introduction of phosphine is continued at a rate which will supply the reaction 10 for a period lasting from one-half to five hours, according to the depth of case desired, after which the delivery of the reagent may be cut off, the apparatus opened up and the goods removed. The case developed upon the goods will 15 appear as a bright, silvery surface. If the temperature of the reaction chamber should rise to above 1400° F. which is above the critical point of the iron or steel, not only would the goods be subject to injury by distortion, but the phosphorized surface metal would appear as a black, brittle case of iron phosphide which does not penetrate the metal, but would be liable to flake or be easily rubbed off. The surfacing would act as iron phosphide does when not alloyed with 20 some other element. Such a coating has been referred to as an "oxy-phosphide" which, in fact, is not a phosphide at all but an oxy-salt of the metal with which the phosphorus reacted.

During the procedure with the apparatus as 30 described in Figure 1, the pressure maintained in the reaction chamber 5 is that produced by submerging the end of the vent pipe 11 in the body of water 12, and which may be regulated by changing the degree of said submergence.

35 In the apparatus shown in Figure 2, the reaction chamber 5a, supplied with gas from cylinders 1a, 2a through valve 3a and pipe 4a, is in the form of an elongated tube closed at its ends and suitable for treating elongated objects, such as rods and pipes. Here, the furnace 6a consists of brickwork heated by fluid fuel burner 1a. The vent pipe 11a dips into the water container 12a, as before. The process here will be substantially as described in connection 45 with Figure 1.

In Figure 3, cylinders 1b, 2b deliver gases under control of valve 3b, through pipe 4b, into a reaction chamber 5b which is in the form of a wheeled vehicle running on track 14 into a furnace 6b which may receive heat from any suitable source typified by hot air pipe 1b leading from a suitable combustion chamber. Chamber 5b is vented by pipe 11b dipping into water receptacle 12b, as in the cases of Figures 1 and 2.

55 Figure 4 shows a form of apparatus in which the gaseous reagent is generated in adjunctive apparatus consisting of phosphine generator 1c discharging into storage gasometer 15, whence gas escapes through pipe 4c past three-way valve 60 3c which also communicates, by way of pipe 2c, with a source of illuminating gas; said valve 3c being made to deliver through pipe 4c' into an elongated reaction chamber 5c enclosed in a furnace 6c heated by electric resistance element 65 7c. Reaction chamber 5c in this instance is vented by pipe 11c dipped into water receptacle 12c, as before. The apparatus shown in Figure 4 is substantially that used in producing the experimental cased articles referred to in this specification. The phosphine was generated in the apparatus, although it is to be noted that commercial phosphine can now be purchased in cylinders, under pressure, such, for instance, as 70 is used in other commercial processes, so that

generation of phosphine in situ may not ordinarily be necessary.

In the use of any of the apparatus disclosed, at the end of the time needed to give the desired iron phosphide conversion on the surface of the article, the reagent gas input is slowed down and the temperature of the reaction chamber increased somewhat to allow the phosphorus to penetrate deeper into the surface. At the end of this last-named period, the tube will be cooled 10 down to below the temperature at which the article would oxidize in air; the flow of phosphine reagent is stopped altogether; the apparatus is again washed out with hydrogen or illuminating gas; and the phosphided or cased article or articles then removed from the reaction chamber.

15 By the method and apparatus herein described, metal objects already fabricated or formed can be made acid and corrosion proof and capable of receiving a high luster.

20 I claim:

1. The process of rendering resistant to deteriorating influences, articles made of metal known to combine with phosphorus to form phosphide which consists in exposing the article, 25 while in the solid state, to the reaction of free or nascent phosphorus in the form of vapor, confined with the article under pressure materially above atmosphere and at a temperature below the critical temperature of the metal of the 30 article but at least as high as the vaporizing point of the phosphorus, oxygen, nitrogen and other volatiles reactive as to the phosphorus being excluded.

2. The process described in claim 1, in which 35 the confined reaction space is initially scavenged to free it from air, and the phosphorus, during the scavenging period is protected by an enveloping medium from which it is releasable by vaporization.

40 3. The process described in claim 1, in which pressure is maintained in the reaction space by confinement of the vapor of the phosphorus.

45 4. The process described in claim 1, in which the said phosphorus reagent is disengaged, under the heat maintained in the reaction, from a phosphide of a metal having less affinity for the phosphorus than the subject metal being converted and presented, in the form of gas, to the metal being treated.

50 5. The process described in claim 1, in which the confined reaction space is primarily scavenged by the delivery thereto of hydrogen gas sufficient in quantity to displace from said space, 55 air or other oxidizing influence which precedes the free or nascent phosphorus therein.

60 6. The process described in claim 1, in which the confined reaction space is primarily scavenged by the delivery thereto of hydrogen gas sufficient in quantity to displace from said space, 60 air or other oxidizing influence which precedes the free or nascent phosphorus therein; the introduced hydrogen gas being supplied in quantity sufficient to reduce oxide scale upon the surface of the subject metal.

65 7. The process described in claim 1, in which the reaction between the phosphorus and the metal is interrupted after but a portion of the subject metal has been converted into its phosphide and thereby leaving a body of non-phosphorized subject metal with a phosphide case united thereto through a diffused region of merger.

70 8. The process described in claim 1, in which the reaction between the phosphorus and the

- metal is interrupted after but a portion of the subject metal has been converted into its phosphide; a body of non-phosphorized subject metal is left with a phosphide case united thereto through a diffused region of merger; and the depth of such case is determined by regulation of the duration of the reaction with the phosphorus and the pressure and temperature maintained in the reaction.
10. The process as described in claim 1, in which the source of the reacting nascent phosphorus is phosphine substantially free from other reactive elements.

10. The process described in claim 1, in which the subject metal is mainly iron, and the converted corrosion resisting portion thereof is mainly iron phosphide.

11. The process described in claim 1, in which the subject metal is mainly iron and the converted corrosion resisting portion thereof is mainly iron phosphide, and in which said process free hydrogen is introduced in quantity sufficient to reduce the scale on the iron and leave the iron subject to reaction with the phosphorus.

ROY B. McCUALEY